

Patented Apr. 17, 1928.

1,666,428

# UNITED STATES PATENT OFFICE.

KARL STOBRAWA, OF GLEIWITZ, GERMANY.

## PROCESS OF PREPARING PIG IRON IN HIGHLY-HEATED MIXERS.

No Drawing. Application filed January 22, 1927, Serial No. 162,932, and in Germany February 16, 1926.

It is well known that the preliminary treatment of liquid pig-iron may be accomplished in the so-called flat hearth mixer by means of the ore preliminary refining process, for the purpose of reducing the percentage of the metalloids Si, Mn, C and P in the pig-iron, thus accelerating the preparation in the final oven, and shortening and equalizing the finishing process in the open

10 hearth or Martin oven as much as possible. It is also well known that in this process shortly after the operation of the flat hearth mixer has commenced, the major portion of manganese besides silicium will be removed 15 from the pig-iron, and mixes with the slag or clinker and therefore will be lost for the process in the finishing oven, whereby the metallurgical course of the finishing process and the quality of the final product may be 20 unfavorably affected. In order to obtain a mixer product having all the required qualities, the pig-iron used for performing said ore refining process should, for the above mentioned reasons, be of a well determined 25 composition, particularly it should be poor in sulphur, that is a special pig-iron which cannot be used for other purposes.

A notable progress in the previous treatment of pig-iron within the flat hearth 30 mixer would consist in that any kind of pig-iron in the trade could be used. In practice it has also been found that the continuous work of preparation accomplished by the flat hearth mixer must be limited in a certain way in order to not affect the security 35 of operation of this mixing oven, as the hearth as well as the walls of the oven will be heavily attacked by a prolonged preparation.

40 Such a mixing product contains among others an average percentage of:

C=about 3-3.5%

Mn=about 0.3-0.4%

Si=about 0.1%.

45 Such a product of flat hearth mixer product is already more convenient for subsequent treatment in the Martin or open hearth oven (liquid process) than pig-iron directly proceeding from blast-furnaces because it 50 contains less slag forming substances. However the refining of such an intermediate product still always requires a considerable addition of oxidizing and calcareous materials, whereby larger quantities 55 of slags or clinkers will be formed which must be carried through the whole process

and will considerably retard the time of the whole process, as the thick layer of slags will prevent an intensive transmission of heat between the metal contents of the oven and the flames of the Martin or open hearth oven. In the proportions in which the percentage of the main slag forming materials, the metalloids C, Mn, P and Si are reduced, I 60 may reduce the oxidizing and calcareous additions and thus obtain a thinner layer of slags more rich in oxide, which secures the necessary conditions for a rapid and intensive progress of the refining process in the finishing oven. It is well known that in 65 the Martin or open hearth oven the full advantages resulting by the applying of the liquid process that is an increased production and reduced expense of coal may be obtained only if a suitable liquid material 70 may be supplied to said Martin or open hearth oven.

In order to prepare such a liquid material, it is suggested according to my present invention to use the flat hearth mixer (highly 80 heated mixer) for the preliminary preparation or treatment of pig-iron; it is well known that said mixer, in contradistinction to any other mixing devices enables heating gases as well as combustion air to be recovered; in order to save the brick work of 85 the oven, avoid the disagreeable corrosion of the hearth thereof, obtain the major portion of manganese of pig-iron, obtain a mixing product with a minimum percentage of 90 slag forming materials and determinate compositions, and increase the production of the flat hearth mixer, all this being attained, according to the invention, by adding to the pig-iron, highly heated pig-iron waste in 95 convenient amounts such pig-iron waste as herein referred to being understood to be low carbon scrap iron.

The addition of cold pig-iron waste to a 100 mixer bath is already known—however in this working method comparatively small quantities of waste iron only can be supplied to the contents of the oven and therefore a slight reduction only of the percentage of metalloids may be obtained. On the other hand owing to the slow smelting of the 105 cold waste iron the major portion of the manganese will be lost by oxidation; it will not be possible to manufacture a product of mixer of the composition hereinafter 110 claimed. The liquefying operation of the previously heated waste iron added to the

- material will be effected extremely rapidly and accomplished in the well known way, that is upon the bringing together of these additions poor in carbon and which separately are not easily fusible, with the metallic contents of the oven of about 2-2.5% of C., the carburation of the previously heated waste iron poor in carbon will be effected immediately whereby the melting temperature thereof will be considerably lowered; therefore the formation of a pig-iron like body will take place, which immediately after its formation will be dissolved in the bath rich in carbon.
- 15 The use of additions poor in carbon in a fluid state (pig-iron waste or the like) for the reduction of the percentage of metalloids in the pig-iron is well known; however the carrying into practical effect of such use requires large devices (converters or Martin ovens) and maximum temperatures, whilst according to my present process the same purpose—reduction of the percentage of metalloids in pig-iron without melting the latter as such—will be attained without it being necessary to melt the waste iron as such, by accumulating most inexpensive heat in the solid additions by means of simple devices and low temperatures and supplying the flat hearth mixer with such heat.

It has also been proposed to make use of iron sponge in the preliminary pig-iron treatment within the mixer; however, for performing the process according to the present invention, such iron sponge cannot be used, because it burns at the preliminary heating at 800 to 1000° C.

As a substitute for the unsafe ore refining process I use according to this invention, in the flat hearth mixer a simple pig-iron waste melting process which does not attack the hearth and walls of the oven, which will increase the production of the mixer, does not drive the manganese contents out from pig-iron into the slag and enables the sulphur to be eliminated from the bath.

For carrying the new process of preliminarily treating pig-iron in the highly heated mixer into practical effect, the pre-heating of the metallic additions (pig-iron waste) is produced by means of a source of heat independent from the Martin or open hearth oven and which operated with most inexpensive heating fluids, such as coal dust, blast-furnace and coke-oven gases and the like, will heat such additions to the highest possible temperature, which however will be below the melting temperature thereof. The more such temperature will be close to the melting temperature, the greater will be the production of the flat hearth mixer and the larger may be quantity of metallic additions, the greater will be the reduction

of carbon in pig-iron. In order to make this new process of preliminarily treating pig-iron continuous, I manufacture for instance in flat hearth mixer of 150 tons first a mixer contents of about 130 tons of pig-iron and previously heated waste ingot-iron of about the following composition:

C=about 2%.  
Mn=about 1.5-2%.

To these mixer contents I add: about 12 tons of liquid pig-iron, about 8 tons of previously heated metallic additions (waste ingot-iron). By the action of the flames in the oven and the heat stored in the mixer contents these previously heated additions will be converted after a short time into a pig-iron like easily liquid body and the new pig-iron added will be brought to a higher temperature. The total contents of 150 tons will then have substantially the same composition as the initial bath:

C=about 2%.  
Mn=about 1.5-2%.

Now about 20 tons of this intermediate product may be taken from the mixer and brought into the finishing oven for subsequent treatment.

Further additions of about 12 tons liquid pig-iron and about 8 tons previously heated waste iron and the removal of a corresponding quantity of about 20 tons from the mixer contents will result into the continuous new flat hearth mixer process. The silicon contents of the pig-iron, as is well known, will be removed from the mixer bath by the action of the basic slag and if necessary by a little oxidizing addition. In the new process of preliminary treating pig-iron the unsafety of operation of the flat hearth mixer will be avoided, the mixer contents may be increased according to requirements and therefore the weight of the mixer charge also.

Having now fully described my said invention, what I claim and desire to secure by Letters Patent, is:

A process for preheating pig-iron in the flat hearth mixer (highly heated mixer) consisting in supplying to the pig-iron, which latter is rich in carbon, low carbon scrap iron preheated at a temperature as close as possible to the melting point by means of a source of heat independent from the mixer, whereby an immediate carburation of said low carbon scrap iron and a lower melting point of same occurs in order to maintain substantially constant the percentage of manganese contained in the pig-iron to be treated and to diminish accordingly the percentage of silicon, carbon and phosphorus.

In testimony whereof I have hereunto set my hand.

KARL STOBRAWA.